

## UNITED STATES PATENT OFFICE

2,121,023

## METHOD OF MOISTUREPROOFING WRAPPING MATERIALS

Ralph T. K. Cornwell, Fredericksburg, Va., assignor to Sylvania Industrial Corporation, Fredericksburg, Va., a corporation of Virginia

No Drawing. Application January 29, 1936,  
Serial No. 61,313

18 Claims. (Cl. 91—68)

The invention relates in general to a moistureproofing composition and to materials coated therewith. More particularly it relates to a wrapping material coated with such a composition which is thereby adapted for use in wrapping moisture-containing products, and to correlated improvements whereby the sealing of such wrapping materials is enhanced through the use of a solvent.

5 There are now in common use a number of non-fibrous cellulosic wrapping materials, some of which are coated with a moistureproofing composition for the purpose of rendering them suitable for wrapping foodstuffs, drugs, tobacco products and the like. When very moist or wet materials such as butter, cheese, meat and the like are packed in such moistureproof wrapping materials, the moistureproof coating frequently becomes loosened from the base and may become detached with the result that the utility of the package is seriously impaired. It has been proposed to increase the adherence of the moistureproof coating to the base sheet material through the use of an intermediate waterproof coating disposed between the moistureproof coating and the base. The use of an intermediate coating requires a double coating operation, expensive solvent mixtures and greatly increases the cost of the wrapping material.

10 Heretofore, it has been proposed to seal moistureproofed wrapping materials by heat and pressure, in which case the effectiveness of the seal depends upon the heat-fusible ingredients of the moistureproofing composition. The seals produced by heat and pressure alone are, however, lacking in strength and tenacity so that such seals are suitable only where there is no substantial strain. It has been proposed, also, to seal moistureproofed wrapping materials by a solvent for the coating, and preferably with heat and pressure. With the moistureproofing compositions heretofore available, the use of a solvent was objectionable in that, instead of rendering the coating composition adhesive, the solvent partially dissolved the coating and loosened it from the base without providing an effective seal. It has been found that the strength of a seal produced by the action of a solvent upon the moistureproofing composition depends in a large measure upon the nature and amount of the several ingredients present in the composition.

15 It is a general object of the present invention to provide a transparent, moistureproof coating composition which, when applied to a suitable base, will enable the contiguous surfaces of the

coated base to be sealed by means of a solvent to provide a strong permanent seal without detracting from the transparency or moistureproofing of the coating.

Another object of the invention is to provide a 5 wrapping material having a moistureproof coating thereon which will enable the contiguous coated surfaces to be sealed together by means of a solvent and pressure and which coating is strongly adherent to the base in the presence of 10 liquid water for a substantial period of time.

It is a further object of the invention to incorporate in a coating composition comprising a lacquer base and a wax, a plasticizing resin which is odorless, substantially colorless, light stable and 15 soluble in lacquer base solvents.

It is a specific object of the invention to provide a novel coating composition adapted for coating sheets and films formed of a hydrophilic colloid, the coating being transparent, moistureproof, non-tacky and strongly adherent to the base and capable of providing a strong permanent seal of contiguous coated surfaces by the use of 20 solvent and pressure.

Other objects of the invention will in part be 25 obvious and will in part appear hereinafter.

The coating composition of the present invention comprises in general a compatible mixture of a lacquer base, a wax, a wax-blending agent, 30 a resin formed by combining an alkyd resin and an aromatic sulphonamide-aldehyde resin and a suitable solvent mixture therefor (said resin will hereinafter be referred to as a plasticizing resin).

To this mixture may be added a plasticizer, a 35 pigment, a dye and/or other lacquer ingredients.

The invention accordingly comprises novel products possessing the characteristics, properties, elements and the relation of elements all as exemplified in the following detailed disclosure and the scope of the application of which will be 40 indicated in the claims.

By way of illustration, but not by way of limiting the invention, it may be stated that the several ingredients may be present in the composition 45 after evaporation of solvent in the following general proportion:

|                                 | Percent        |
|---------------------------------|----------------|
| Lacquer base                    | from 40 to 65  |
| Plasticizing resin              | from 5 to 35   |
| Plasticizer                     | from 5 to 10   |
| Wax                             | from 0.5 to 7  |
| Non-volatile wax blending agent | from 0.5 to 30 |

For the lacquer base there may be employed a 55

suitable cellulose derivative such, for example, as nitrocellulose, cellulose acetate, ethyl cellulose, benzyl cellulose or a film-forming synthetic resin such as a polymerized vinyl resin, a chlorinated diphenyl resin, and the like. In the now preferred embodiment of the invention, the lacquer base comprises nitrocellulose. The plasticizing resin distinguishes over the lacquer base resins in that it has substantially no film-forming properties when used alone.

The plasticizing resin used in the invention may be produced as above stated. The alkyd resin is made by reacting a polyhydric alcohol such, for example, as glycol or glycerol with a polycarboxylic acid such, for example, as maleic acid or phthalic acid. The alkyd resin is combined or reacted with an aromatic sulphonamide-aldehyde resin formed by the condensation of an aromatic sulphonamide, as benzene sulphonamide, with an aldehyde, for example, formaldehyde. The product resulting from the condensation of the two resins is a viscous liquid or soft solid, which is characterized by being light in color, substantially transparent, odorless, water-repellent, substantially light-stable, soluble in common lacquer solvents, and which functions to improve the flexibility of coatings and films produced from compositions containing it. A more important feature of the plasticizing resin is that it renders the coatings or films solvent-sealable with a like film to produce a joint which is stronger than a similar joint produced when said film is heat-sealed and stronger than a joint produced with the same solvent on films formed from the same composition omitting the plasticizing resin.

As a plasticizer there may be used either per se or in combination ethoxy ethyl phthalate, dibutyl phthalate, triphenyl phosphate, butyl benzoyl benzoate and the like.

Any suitable animal, mineral or vegetable wax may be used to impart moistureproofness to the composition, but in the preferred embodiment of the invention there is used paraffin wax having a high melting point.

The non-volatile wax blending agent may be a blown oil and/or a gum or resin. Either a blown or boiled oil of animal or vegetable origin may be employed, for example, rapeseed, neat's-foot, linseed, soya bean, perilla, etc. The gum or resin used as a wax-blending agent may be of the type of wax-free dammar or an ester gum; also phthalates of hydroxy fatty acids and other materials which are characterized by having a low melting point and a solubility both in hydrocarbon and in oxygen-containing solvents used in the lacquers may be utilized. In the preferred embodiment, the wax-blending agent contains a blown oil and a resin.

By way of more specific illustration of an improved moistureproofing composition embodying my invention, I mention the following examples in which all ingredients, except the solvents are expressed in parts by weight:

|                           | No. 1 | No. 2 | No. 3 | No. 4 | No. 5 |
|---------------------------|-------|-------|-------|-------|-------|
| Nitrocellulose (5-6 sec.) | 45    | 30    | 50    | 40    | 45    |
| Plasticizing resin        | 20    | 30    | 35    | 35    | 22    |
| Di-butyl phthalate        | 10    | 5     | 4     | 4½    | 5     |
| Paraffin, M. P. 67° C.    | 5     | 5     | 4     | 4½    | 5     |
| Dammar gum                |       | 30    |       | 20    |       |
| Ester gum                 | 20    |       | 10    |       | 20    |
| Blown rapeseed oil        |       |       | 1     | ½     | ½     |

A lacquer may be prepared by taking up about 75 10 parts of one of the above compositions in

about 250 parts of a suitable solvent, e. g., one consisting of 15% ethyl acetate, 15% butyl acetate and 70% toluene. This solution may then be applied as a coating and dried in a heated dryer in the usual way, or formed into sheets or films, etc. if desired.

These novel compositions may be used in a number of arts, but are particularly advantageous for coating wrapping materials formed of transparent, organic plastic materials such as cellulose derivatives and synthetic resins, on account of the fact that the films deposited upon evaporation of solvent are transparent, non-greasy, non-tacky, substantially odorless and highly moisture-proof.

Further the compositions are especially adapted for coating wrapping materials formed of organic hydrophilic colloids such, for example, as cellulose hydrate, alkali-soluble cellulose ethers, gelatin, casein and the like. On such materials, the coating effectively prevents the diffusion of water vapor through the material and, at the same time, shows a high waterproofness and strong adherence to the base in the presence of liquid water. As a result of these characteristics, a wrapping material comprising a sheet of a hydrophilic colloid and coated with the moistureproofing composition of the invention is especially adapted for wrapping various types of moisture-containing goods, for example, foodstuffs as meat, butter, cheese, as well as drugs, tobacco and the like.

I have found that if a film or sheet of glycerinated regenerated cellulose having a thickness of about one-thousandth of an inch be coated, preferably on each side, with a moistureproofing composition of approximately 1.5 ten thousandth of an inch total thickness prepared in accordance with the present invention, the resistance of the coated sheet to the diffusion of water vapor is at least 50 times as great as that of the uncoated sheet of glycerinated regenerated cellulose when both are tested comparatively at ordinary temperatures up to 38° or 40° C. The term "moisture-proof" as used herein is intended to cover a composition having such a moisture proofing value when so tested.

Another outstanding characteristic of the wrapping materials coated with the moistureproofing composition of the invention is that the contiguous surfaces may be effectively sealed together by the application of a solvent sealing agent such as methyl "Cellosolve", methyl acetate, acetone, etc. When a small amount of the solvent is applied to the contiguous, coated surfaces and the surfaces pressed together, preferably with the application of heat, there is produced, after evaporation of the sealing solvent, a strong tenacious seal without impairing the transparency, flexibility or moistureproofness of the coating. The seal so produced is materially stronger than a seal of the same dimensions produced by heat-sealing analogous, moistureproof, transparent coatings of the same thickness when applied to the same base sheet material.

Since certain changes may be made in the above composition of matter and article produced utilizing the same, and different embodiments of the invention could be made without departing from the scope thereof, it is intended that all matter contained in the above description shall be interpreted as illustrative and not in a limiting sense.

It is also to be understood that the following claims are intended to cover all of the generic and specific features of the invention herein de-

scribed, and all statements of the scope of the invention which, as a matter of language, might be said to fall therebetween.

I claim:

- 5 1. A moistureproofing composition comprising a lacquer base, a wax, a wax-blending agent and a plasticizing resin resulting from the condensation of an alkyd resin with a sulphonamide-aldehyde resin.
- 10 2. A moistureproofing composition comprising a lacquer base, a wax, a wax-blending agent, a plasticizing resin resulting from the condensation of an alkyd resin with a sulphonamide-aldehyde resin and a solvent, said ingredients being present in such proportions as to deposit, upon evaporation of solvent, a transparent, moisture-proof film which is solvent-sealable with a like film to produce a joint which is stronger than a similar joint produced when said films are heat-sealed.
- 15 3. A moistureproofing composition comprising a lacquer base, a wax, a wax-blending agent, a plasticizing resin resulting from the condensation of an alkyd resin with a sulphonamide-aldehyde resin, a plasticizer and a solvent, said ingredients being present in such proportions as to deposit, upon evaporation of solvent, a flexible, transparent, moistureproof film which is solvent-sealable with a like film to produce a joint which is stronger than a similar joint produced when said films are heat-sealed.
- 20 4. A moistureproofing composition comprising a lacquer base resin, a wax, a wax-blending agent, a plasticizing resin resulting from the condensation of an alkyd resin with a sulphonamide-aldehyde resin, a plasticizer and a solvent, said ingredients being present in such proportions as to deposit, upon evaporation of solvent, a flexible, transparent, moistureproof film which is solvent-sealable with a like film to produce a joint which is stronger than a similar joint produced when said films are heat-sealed.
- 25 5. A moistureproofing composition comprising a cellulose derivative, a wax, a wax-blending agent, a plasticizing resin resulting from the condensation of an alkyd resin with a sulphonamide-aldehyde resin, a plasticizer and a solvent, said ingredients being present in such proportions as to deposit, upon evaporation of solvent, a flexible, transparent, moistureproof film which is solvent-sealable with a like film to produce a joint which is stronger than a similar joint produced when said films are heat-sealed.
- 30 6. A moistureproofing composition comprising nitro-cellulose, a wax, a wax-blending agent containing a blown oil and a gum, a plasticizing resin resulting from the condensation of an alkyd resin with a sulphonamide-aldehyde resin, a plasticizer and a solvent, said ingredients being present in such proportions as to deposit, upon evaporation of solvent, a flexible, transparent, moistureproof film which is solvent-sealable with a like film to produce a joint which is stronger than a similar joint produced when said films are heat-sealed.
- 35 7. A moistureproofing composition comprising 40% to 65% of a lacquer base, 0.5% to 7% of a wax, 0.5% to 30% of a wax-blending agent, 5% to 35% of a plasticizing resin resulting from the condensation of an alkyd resin with a sulphonamide-aldehyde resin, 5% to 10% of a plasticizer and a solvent, said ingredients being present in such proportions as to deposit, upon evaporation of solvent, a flexible, transparent, moistureproof film which is solvent-sealable with a like film to

produce a joint which is stronger than a similar joint produced when said films are heat-sealed.

8. A moistureproofing composition comprising 40% to 65% of nitrocellulose, 0.5% to 7% of paraffin wax, 0.5% to 30% of a wax-blending agent containing a blown oil and a gum, 5% to 35% of a plasticizing resin resulting from the condensation of an alkyd resin with a sulphonamide-aldehyde resin, 5% to 10% of a plasticizer and a solvent mixture, said ingredients being present in such proportions as to deposit, upon evaporation of solvent, a flexible, transparent, moistureproof film which is solvent-sealable with a like film to produce a joint which is stronger than a similar joint produced when said films are heat-sealed.

9. As an article of manufacture, a non-fibrous organic hydrophilic colloid material having a moistureproof coating comprising a lacquer base, a wax, a wax-blending agent and a plasticizing resin resulting from the condensation of an alkyd resin with a sulphonamide-aldehyde resin, said coating being solvent-sealable with a like coating to produce a joint which is stronger than a similar joint produced when said coatings are heat-sealed.

10. As an article of manufacture, a non-fibrous cellulosic material having a moistureproof coating comprising a lacquer base, a wax, a wax-blending agent, a plasticizing resin resulting from the condensation of an alkyd resin with a sulphonamide-aldehyde resin, and a plasticizer, said coating being solvent-sealable with a like coating to produce a joint which is stronger than a similar joint produced when said coatings are heat-sealed.

11. As an article of manufacture, regenerated cellulose having a moistureproof coating comprising a lacquer base, a wax, a wax-blending agent, a plasticizing resin resulting from the condensation of an alkyd resin with a sulphonamide-aldehyde resin, and a plasticizer, said coating being solvent-sealable with a like coating to produce a joint which is stronger than a similar joint produced when said coatings are heat-sealed.

12. As an article of manufacture, a wrapping material having a moistureproof coating comprising a lacquer base, a wax, a wax-blending agent and a plasticizing resin resulting from the condensation of an alkyd resin with a sulphonamide-aldehyde resin, said coating being solvent-sealable with a like coating to produce a joint which is stronger than a similar joint produced when said coatings are heat-sealed.

13. As an article of manufacture, a wrapping material comprising a transparent sheet of non-fibrous, cellulosic material having a moistureproof coating comprising a lacquer base, a wax, a wax-blending agent, a plasticizing resin resulting from the condensation of an alkyd resin with a sulphonamide-aldehyde resin, and a plasticizer, said coating being solvent-sealable with a like coating to produce a joint which is stronger than a similar joint produced when said coatings are heat-sealed.

14. As an article of manufacture, a wrapping material comprising a transparent sheet of regenerated cellulose having a moistureproof coating comprising a lacquer base, a wax, a wax-blending agent, a plasticizing resin resulting from the condensation of an alkyd resin with a sulphonamide-aldehyde resin and a plasticizer, said coating being solvent-sealable with a like coating to produce a joint which is stronger than a similar joint produced when said coatings are heat-sealed.

joint produced when said coatings are heat-sealed.

15. As an article of manufacture, a wrapping material comprising a transparent sheet of non-fibrous, organic hydrophilic colloid material having a moistureproof coating comprising a cellulose derivative, a wax, a wax-blending agent, a plasticizing resin resulting from the condensation of an alkyd resin with a sulphonamide-aldehyde resin, and a plasticizer, said coating being solvent-sealable with a like coating to produce a joint which is stronger than a similar joint produced when said coatings are heat-sealed.
16. As an article of manufacture, a wrapping material comprising a transparent sheet of regenerated cellulose having a thin moistureproof coating comprising nitrocellulose, a wax, a wax-blending agent containing a blown oil and a gum, a plasticizing resin resulting from the condensation of an alkyd resin with a sulphonamide-aldehyde resin, and a plasticizer, said coating being solvent-sealable with a like coating to produce a joint which is stronger than a similar joint produced when said coatings are heat-sealed.
17. As an article of manufacture, a wrapping

material comprising a transparent sheet of regenerated cellulose having a thin moistureproof coating comprising 40% to 65% of a lacquer base, 0.5% to 7% of a wax, 0.5% to 30% of a wax-blending agent, 5% to 35% of a plasticizing resin resulting from the condensation of an alkyd resin with a sulphonamide-aldehyde resin, and 5% to 10% of a plasticizer, said coating being solvent-sealable with a like coating to produce a joint which is stronger than a similar joint produced when said coatings are heat-sealed.

18. As an article of manufacture, a wrapping material comprising a transparent sheet of regenerated cellulose having a thin moistureproof coating comprising 40% to 65% of nitrocellulose, 0.5% to 7% of paraffin wax, 0.5% to 30% of a wax-blending agent containing a blown oil and a gum, 5% to 35% of a plasticizing resin resulting from the condensation of an alkyd resin with a sulphonamide-aldehyde resin, and 5% to 10% of a plasticizer, said coating being solvent-sealable with a like coating to produce a joint which is stronger than a similar joint when said coatings are heat-sealed.

RALPH T. K. CORNWELL. 25